

149

Patented Aug. 4, 1931

1,816,860

## UNITED STATES PATENT OFFICE

GEORGE L. MAGOUN AND DEAL H. TOMPKINS, OF NITRO, WEST VIRGINIA, ASSIGNEES  
TO THE RUBBER SERVICE LABORATORIES COMPANY, OF AKRON, OHIO, A CORPO-  
RATION OF OHIO

## METAL PICKLING PROCESS

Application filed November 6, 1930. Serial No. 493,907.

The present invention relates to the cleaning and preservation of metallic surfaces, wherein the metal is in contact with a liquid of an acid nature. More particularly, 5 the invention relates to the prevention of excessive pitting and embrittlement of a metal when subjected to a pickling process by treatment with a dilute solution of a non-oxidizing acid.

10 Certain objects of the present invention are to prevent the acid pickle liquor from attacking clean portions of the surface of a metal; to obviate over-pickling, embrittlement and pitting of the articles treated; to minimize the amount of metal lost in pickling; to increase the efficiency of the pickling operation; to prolong the effective life 15 of the pickling bath; and particularly to facilitate the pickling operation. Other 20 and further objects of the invention will be apparent from the following description and accompanying examples.

In the art of pickling, the metal is treated with a dilute acid to remove oxides such as 25 rust, scale, and other deposits, after which the metal is preferably washed with water and dipped into an alkaline bath to remove the last traces of free acid. The acid removes the rust and scale, but unfortunately, 30 from the pickling standpoint, unless some agent to prevent such action is present, it attacks the cleaned metal itself thereby causing loss of metal and producing an evolution of hydrogen gas, which escapes into 35 the air, carrying with it a fine spray of the acid liquor from the pickling bath and producing an atmosphere possessing corrosive properties and one which is injurious to health and damaging to equipment.

40 By the present invention, these objectionable features of the pickling process are substantially overcome or reduced to a minimum. To accomplish to as great an extent as possible the objects set forth in accordance 45 with the present invention, there is

added to the pickling bath, a regulating agent or ingredient which acts to restrain the action of the acid from attacking clean metal but assists in removing the rust, scale and other deposits, or in other words the regulator or inhibitor causes the acid selectively to remove such materials without appreciably attacking the clean portions of the metal under treatment.

50 The pickle regulator or inhibitor, as disclosed in the present application, comprises an acid derivative of a reaction product of a thiourea and an aldehyde-ammonia; that is, a product formed by first reacting an aldehyde with ammonia, then further reacting a thiourea therewith, and treating the product so obtained with an acid of any concentration necessary to produce chemical combination at the reaction temperature employed.

55 In the examples hereinafter set forth for carrying out the metal pickling process, conditions were imposed which duplicated, so far as possible, those commonly followed in commercial practice, so far as concerned acid 60 concentrations and temperatures employed.

65 Test pieces of 30 gauge cold rolled tin plate steel stock, approximately 4" x 3" in dimension, were immersed in approximately 750 c. c. of a water solution of sulfuric acid containing approximately 6% by weight of 66° Bé. acid to which had been added a small quantity of one of the preferred type of inhibitors. The loss in weight 70 of the steel test pieces resulting from maintaining the strips in the pickle bath in the manner described for a definite period of time was then determined. The temperature of the pickling bath was maintained at from 75 83 to 84° C. For the acid concentration 80 set forth, commercial practice is to pickle at approximately 66 to 88° C. The results so obtained were compared with similar tests 85 wherein the steel pieces were subjected, under the conditions set forth, to the action of 90

an acid solution of the strength and for the time specified above, but containing no inhibitor.

One method whereby one of the preferred class of compounds, for example a sulfuric acid derivative of a reaction product of thiocarbanilide and acetaldehyde-ammonia, was prepared as follows:

Substantially two molecular proportions 10 of acetaldehyde were dissolved in an organic solvent, for example, a quantity of ethyl alcohol equal to approximately three times the weight of the acetaldehyde. Ammonia, preferably in the anhydrous condition, was 15 passed thereinto until substantially two molecular proportions of the gas was absorbed as indicated by the increase in weight, while agitating and maintaining a temperature preferably not higher than 25° C. To 20 the product thus formed, substantially one molecular proportion of thiocarbanilide was added and the mixture heated to and maintained at a refluxing temperature while agitating until the reaction was complete. The 25 solvent employed, for example ethyl alcohol, was then removed preferably by distillation. The residual product thus formed, consisting of a thick viscous resin, was then 30 treated with substantially one molecular proportion of sulfuric acid, preferably in the form of approximately 93% acid, and the product thus formed heated in a convenient manner, at a temperature preferably of substantially 100 to 110° C. for a 35 period of approximately 24 hours. The final product thus formed was a hard, brittle resin which formed a fine powder when ground that was readily and completely soluble in a pickle liquor, as for example 40 dilute sulfuric acid.

A sample of the product prepared as described above was incorporated in a pickling bath in the manner hereinbefore described. Thus, a steel test piece, 3" x 4" 45 in dimension, cut from 30 gauge cold rolled tin plate stock, exposing approximately 24 square inches of surface and weighing 17.5105 grams, was found to lose but 0.0285 grams after 40 minutes pickling in 750 c. c. 50 of a 6% sulfuric acid solution containing 0.07 grams of the inhibiting product hereinbefore described. A similar test piece weighing 18.2050 grams and treated in the same manner, but without the use of any 55 inhibitor, lost 8.5350 grams. Thus it is shown that when the sulfuric acid derivative of the reaction product of thiocarbanilide and acetaldehyde-ammonia is employed as 60 an inhibitor, the loss in weight per square inch of surface exposed corresponds to 0.00119 grams, whereas when no inhibitor is employed in the test described, the loss per square inch of surface exposed corre- 65 sponds to 0.35600 grams. The loss in weight

per square inch of surface exposed is only 0.33 percent as great by employing the inhibitor set forth as results if no inhibitor is employed in the pickling process. A greater saving in metal losses results from 70 the use of a large amount of the inhibitor than that employed in the example. Moreover, the steel plates pickled in the presence of the inhibitor set forth are clean and not stained upon removal from the bath. 75

Other acid derivatives of a reaction product of a thiourea and an aldehyde-ammonia have been prepared in a manner analogous to that hereinbefore set forth and tested as 80 inhibitors in a pickling bath in the manner hereinbefore described. Thus, the following products were so prepared and tested:

*Compound A.*—Sulfuric acid derivatives of the reaction product of substantially one molecular proportion of thiocarbanilide and 85 substantially two molecular proportions of butyraldehyde-ammonia.

*Compound B.*—Sulfuric acid derivative of the reaction product of substantially one molecular proportion of thiocarbanilide and 90 substantially two molecular proportions of crotonaldehyde-ammonia.

*Compound C.*—Sulfuric acid derivative of the reaction product of substantially one molecular proportion of thiocarbanilide and 95 substantially two molecular proportions of heptaldehyde-ammonia.

*Compound D.*—Sulfuric acid derivative of the reaction product of substantially one molecular proportion of thiocarbanilide and 100 substantially two molecular proportions of formaldehyde-ammonia.

*Compound E.*—Sulfuric acid derivative of the reaction product of substantially one molecular proportion of thiocarbanilide and 105 substantially two molecular proportions of alpha-ethyl-beta-propyl-acrolein - ammonia.

*Compound F.*—Sulfuric acid derivative of the reaction product of substantially one molecular proportion of thiourea and 110 substantially two molecular proportions of acetaldehyde-ammonia.

*Compound G.*—Sulfuric acid derivative of the reaction product of substantially one molecular proportion of di-ortho-tolyl-thiourea and substantially two molecular proportions of acetaldehyde-ammonia. 115

*Compound H.*—Sulfuric acid derivative of the reaction product of substantially one molecular proportion of phenyl-ortho-tolyl-thiourea and substantially two molecular proportions of acetaldehyde-ammonia. 120

*Compound I.*—Sulfuric acid derivative of the reaction product of substantially one molecular proportion of mono-phenyl-thiourea and substantially two molecular proportions of acetaldehyde-ammonia. 125

*Compound J.*—Sulfuric acid derivative of the reaction product of substantially one molecular proportion of phenyl-piperidyl- 130

thiourea and substantially two molecular proportions of acetaldehyde-ammonia.

5 *Compound K.*—Sulfuric acid derivative of the reaction product of substantially one molecular proportion of phenyl-alpha-naphthyl-thiourea and substantially two molecular proportions of acetaldehyde-ammonia.

10 *Compound L.*—Hydrochloric acid derivative of the reaction product of substantially one molecular proportion of thiocarbanilide and substantially two molecular proportions of acetaldehyde-ammonia.

15 *Compound M.*—Phosphoric acid derivative of the reaction product of substantially one molecular proportion of thiocarbanilide and substantially two molecular proportions of acetaldehyde-ammonia.

20 *Compound N.*—Acetic acid derivative of the reaction product of substantially one molecular proportion of thiocarbanilide and substantially two molecular proportions of acetaldehyde-ammonia.

25 *Compound O.*—Oxalic acid derivative of the reaction product of substantially one molecular proportion of thiocarbanilide and substantially two molecular proportions of acetaldehyde-ammonia.

30 The results of the tests obtained on immersing steel test strips of 30 gauge cold rolled tin plate stock, 3" x 4" in dimension, for 40 minutes in 750 c. c. of 6% by weight of 66° Bé. sulfuric acid at 83° C. in the presence of the indicated quantity of one of the above described inhibitors, are given in 35 Table I.

Table I

| 40 | Inhibiting compound employed | Weight of inhibitor employed | Weight of steel strip before pickling | Weight of steel strip after pickling | Weight loss in grams per sq. inch of surface exposed |
|----|------------------------------|------------------------------|---------------------------------------|--------------------------------------|------------------------------------------------------|
|    |                              | grams                        | grams                                 | grams                                | grams                                                |
| 45 | Compound A                   | 0.07                         | 18.0335                               | 18.0005                              | 0.00137                                              |
|    | Compound B                   | 0.07                         | 17.8082                               | 17.7740                              | 0.00142                                              |
|    | Compound C                   | 0.07                         | 17.9498                               | 17.9415                              | 0.00035                                              |
|    | Compound D                   | 0.07                         | 17.9415                               | 17.9280                              | 0.00056                                              |
|    | Compound E                   | 0.07                         | 17.9370                               | 17.9070                              | 0.00125                                              |
|    | Compound F                   | 0.07                         | 17.3640                               | 17.3425                              | 0.00090                                              |
|    | Compound G                   | 0.07                         | 17.8335                               | 17.8165                              | 0.00071                                              |
|    | Compound H                   | 0.07                         | 17.3235                               | 17.3062                              | 0.00072                                              |
|    | Compound I                   | 0.07                         | 17.8165                               | 17.7995                              | 0.00071                                              |
|    | Compound J                   | 0.07                         | 17.0737                               | 17.0471                              | 0.00111                                              |
|    | Compound K                   | 0.07                         | 17.9950                               | 17.9760                              | 0.00082                                              |
|    | Compound L                   | 0.07                         | 18.6535                               | 18.6251                              | 0.00118                                              |
|    | Compound M                   | 0.07                         | 17.7737                               | 17.7520                              | 0.00090                                              |
|    | Compound N                   | 0.07                         | 17.8746                               | 17.8557                              | 0.00079                                              |
|    | Compound O                   | 0.07                         | 17.9028                               | 17.8752                              | 0.00115                                              |
|    | None                         | None                         | 18.2050                               | 9.6700                               | 0.35600                                              |

55 It is thus apparent from the data set forth that the preferred class of materials constitutes an important and highly efficacious group of inhibitors, as in all cases wherein one of the preferred inhibiting com-

60 pounds was incorporated in the pickle liquid, there resulted a great saving in the loss in weight of the steel test strips as compared with that resulting when no inhibitor was employed.

65 It has further been found that other

ratios of acid, thiourea and aldehyde-ammonia than those hereinbefore set forth may be reacted, and the reaction products so obtained employed as inhibitors. Thus, approximately one molecular proportion of the reaction product of substantially one molecular proportion of thiocarbanilide and substantially two molecular proportions of acetaldehyde-ammonia has been reacted with substantially one and two-thirds molecular proportions of sulfuric acid. The compound thus produced was incorporated in a pickle liquor in the manner hereinbefore described, the amount of inhibitor employed, the bath, and the size and grade of steel sheets used being the same as in the hereinbefore described tests. A steel sheet weighing 18.3820 grams was found after pickling 40 minutes to have lost but 0.0225 grams, or 0.00094 grams per square inch of surface exposed. A sheet of the same stock weighing 18.2050 grams and treated in the same manner, but with no inhibitor present, suffered a loss of 8.5350 grams or 0.35600 grams per square inch of surface exposed.

70 Other modes of employing inhibitors of the class hereinbefore set forth in the acid pickling of metals are apparent to those skilled in the art to which this invention pertains. The products described additionally may be employed in the presence of foaming agents, ionizable substances or other materials ordinarily used, and are employable with the various acids commonly employed commercially in the acid pickling of metals.

75 What is claimed is:

1. A process of pickling a metal which comprises subjecting the metal to be pickled to the action of a substantially non-oxidizing mineral acid solution containing a small proportion of an acid derivative of a reaction product of a thiourea and an aldehyde-ammonia.

80 2. A process of pickling a metal which comprises subjecting the metal to be pickled to the action of a substantially non-oxidizing mineral acid solution containing a small proportion of an acid derivative of a reaction product of a thiourea and an aliphatic aldehyde-ammonia.

85 3. A process of pickling iron and steel products which comprises subjecting the metal to be pickled to the action of a sulfuric acid solution containing a small proportion of an acid derivative of a reaction product of a thiourea and an aldehyde-ammonia.

90 4. A process of pickling iron and steel products which comprises subjecting the metal to be pickled to the action of a sulfuric acid solution containing a small proportion of an acid derivative of a reaction product of a thiourea and an aliphatic aldehyde-ammonia.

5. A process of pickling iron and steel products which comprises subjecting the metal to be pickled to the action of a sulfuric acid solution containing a small proportion of a sulfuric acid derivative of a reaction product of a thiourea and an aliphatic aldehyde-ammonia.
6. A process of pickling iron and steel products which comprises subjecting the metal to be pickled to the action of a sulfuric acid solution containing a small proportion of a sulfuric acid derivative of a reaction product of thiocarbanilide and an aliphatic aldehyde-ammonia.
- 10 7. A process of pickling iron and steel products which comprises subjecting the metal to be pickled to the action of a sulfuric acid solution containing a small proportion of a sulfuric acid derivative of a reaction product of thiocarbanilide and acetaldehyde-ammonia.
- 15 8. A process of pickling iron and steel products which comprises subjecting the metal to be pickled to the action of a sulfuric acid solution containing a small proportion of a product formed by reacting substantially one molecular proportion of thiocarbanilide with substantially two molecular proportions of acetaldehyde-ammonia and further reacting the product thus formed with substantially one molecular proportion of sulfuric acid.
- 20 9. A pickling bath for metal products which comprises a substantially non-oxidizing mineral acid solution containing a small proportion of an acid derivative of a reaction product of a thiourea and an aldehyde-ammonia.
- 25 10. A pickling bath for metal products which comprises a substantially non-oxidizing mineral acid solution containing a small proportion of an acid derivative of a reaction product of a thiourea and an aliphatic aldehyde-ammonia.
- 30 11. A pickling bath for iron and steel products comprising a sulfuric acid solution containing a small proportion of an acid derivative of a reaction product of a thiourea and an aldehyde-ammonia.
- 35 12. A pickling bath for iron and steel products comprising a sulfuric acid solution containing a small proportion of an acid derivative of a reaction product of a thiourea and an aliphatic aldehyde-ammonia.
- 40 13. A pickling bath for iron and steel products comprising a sulfuric acid solution containing a small proportion of a sulfuric acid derivative of a reaction product of a thiourea and an aliphatic aldehyde-ammonia.
- 45 14. A pickling bath for iron and steel products comprising a sulfuric acid solution containing a small proportion of a sulfuric acid derivative of a reaction product of a thiourea and an aliphatic aldehyde-ammonia.
- 50 15. A pickling bath for iron and steel products comprising a sulfuric acid solution containing a small proportion of a sulfuric acid derivative of a reaction product of thiocarbanilide and an aliphatic aldehyde-ammonia.
- 55 16. A pickling bath for iron and steel products comprising a sulfuric acid solution containing a small proportion of a product formed by reacting substantially one molecular proportion of thiocarbanilide with substantially two molecular proportions of acetaldehyde-ammonia and further reacting the product thus formed with substantially one molecular proportion of sulfuric acid.
- 60 17. A process of pickling iron and steel products which comprises subjecting the metal to be pickled to the action of a sulfuric acid solution containing a small proportion of an acid derivative of a reaction product of an aryl substituted thiourea and an aliphatic aldehyde-ammonia.
- 65 18. A process of pickling iron and steel products which comprises subjecting the metal to be pickled to the action of a sulfuric acid solution containing a small proportion of an acid derivative of a reaction product of a di-aryl substituted thiourea and an aliphatic aldehyde-ammonia.
- 70 19. A process of pickling iron and steel products which comprises subjecting the metal to be pickled to the action of a sulfuric acid solution containing a small proportion of a sulfuric acid derivative of a reaction product of an aryl substituted thiourea and an aliphatic aldehyde-ammonia.
- 75 20. A process of pickling iron and steel products which comprises subjecting the metal to be pickled to the action of a sulfuric acid solution containing a small proportion of a sulfuric acid derivative of a reaction product of a di-aryl substituted thiourea and an aliphatic aldehyde-ammonia containing less than eight carbon atoms.
- 80 21. A pickling bath for iron and steel products comprising a sulfuric acid solution containing a small proportion of an acid derivative of a reaction product of an aryl substituted thiourea and an aliphatic aldehyde-ammonia.
- 85 22. A pickling bath for iron and steel products comprising a sulfuric acid solution containing a small proportion of an acid derivative of a reaction product of a di-aryl substituted thiourea and an aliphatic aldehyde-ammonia.
- 90 23. A pickling bath for iron and steel products comprising a sulfuric acid solution containing a small proportion of a sulfuric acid derivative of a reaction product of an aryl substituted thiourea and an aliphatic aldehyde-ammonia.
- 95 24. A pickling bath for iron and steel products comprising a sulfuric acid solution containing a small proportion of a sulfuric acid derivative of a reaction product of thiocarbanilide and acetaldehyde-ammonia.

## 252. COMPOSITIONS,

149

5

1,816,860

products comprising a sulfuric acid solution containing a small proportion of a sulfuric acid derivative of a reaction product of a di-aryl substituted thiourea and an aliphatic aldehyde-ammonia containing less than 5 eight carbon atoms.

In testimony whereof we hereunto affix our signatures.

GEORGE L. MAGOUN.  
DEAL H. TOMPKINS.

10

15

20

25

30

35

40

45

50

55

60

65